

(No Model.)

E. S. EARLEY.

BURIAL CASKET.

No. 298,953.

Patented May 20, 1884.

Fig. 1.



Fig. 2.



Fig. 3.



WITNESSES:

A. P. Grant  
H. F. Kirches

INVENTOR:  
Edward S. Earley,  
BY John A. Federheim.  
ATTORNEY.

# UNITED STATES PATENT OFFICE.

EDWARD S. EARLEY, OF PHILADELPHIA, PENNSYLVANIA.

## BURIAL-CASKET.

SPECIFICATION forming part of Letters Patent No. 298,953, dated May 20, 1884.

Application filed March 26, 1884. (No model.)

*To all whom it may concern:*

Be it known that I, EDWARD S. EARLEY, a citizen of the United States, residing in the city and county of Philadelphia, State of Pennsylvania, have invented a new and useful Improvement in Burial Cases or Caskets, which improvement is fully set forth in the following specification and accompanying drawings, in which—

10 Figure 1 is a plan view, partly broken away, of a burial case or casket embodying my invention. Fig. 2 is a side elevation, partly broken away. Fig. 3 is a vertical section in line *xx*, Fig. 2.

15 Similar letters of reference indicate corresponding parts in the several figures.

My invention consists of a method of making a burial case or casket which is water and air tight, strong and durable, and preservative in its nature, as will be hereinafter fully set forth.

Referring to the drawings, A represents the body of the case or casket, and B the lid thereof. The body and the lid are formed of pieces, 25 *a*, of wood which is saturated with asphalt, coated inside and outside with paper, *b*, known as "felt paper," and an exterior coating of asphalt or other varnish. The bottom *c* of the body is similarly formed, excepting that the 30 under side is well coated with pitch instead of varnish, said bottom being nailed or screwed to battens *C*, which are firmly secured to the body on the inside thereof near the lower end.

D represents battens which are firmly secured to the top of the body on the inside thereof, their upper faces being grooved or channeled, as at *d*, to receive the tongue *d'*, formed on the under side of the lid B, the groove *d* being adapted to contain a proper 35 fluid or material for sealing the joint of the body and lid. Rising from the corners of the body are posts E, which rest on the bottom battens, C, and are in contact with the under side of the upper battens, D, thus assisting to 40 sustain said battens, said posts being secured to the sides of the body or to the upper and lower battens, or both. The battens and posts are coated with asphalt and covered with felt paper; and the upper battens, and lower ones, 45 if desired, are secured to the body by bolts, the openings in the body to receive the heads of said bolts being countersunk and filled with asphalt or equivalent material to cover said

heads. The body and lid are provided with catches, which may be self-fastening; but other means for connecting them may be adopted, it being desirable to force the lid tightly on the bottom and retain it in such condition and position to insure the sealing joint. 55

In the manufacture of the case or casket, 60 the wood is heated and coated with asphalt, some of which enters the pores thereof. The felt paper is then applied, and a hot iron or tool is passed over the paper, pressing the hot paper against the wood, whereby the asphalt on the surface of the wood saturates the paper, and thoroughly incorporates the said asphalt and the paper, and unites the same with the wood. As the wood is saturated with asphalt and coated with asphalt, with a covering of asphalt-saturated felt paper, some 65 of the asphalt and the paper becoming almost homogeneous, it is evident that the wood is rendered exceedingly durable and preserved 70 from the injurious effects of water, air, and ground, the joints being close and tight, and preventing the entrance of water therethrough. The exterior coating of varnish serves both as a finish and an additional protection to the case or casket. The case or 75 casket, owing to the nature of the saturation of the wood and coated paper, acts as a preservative to the contents of the same.

The case or casket is more specially designed as an outer case and a substitute for 80 expensive cedar boxes and vaults, while possessing the several advantages stated.

Having thus described my invention, what I claim as new, and desire to secure by Letters Patent, is—

90 The method of protecting the body and lid of a burial-casket, consisting in forming the same of wood, heating the wood, coating it with asphalt, applying felt paper to the wood, and running a hot iron or tool over the paper, 95 pressing the hot paper against the wood, whereby the wood and paper become saturated with asphalt, and the paper is united to the wood, the asphalt of the wood and of the paper becoming homogeneous, substantially 100 as and for the purpose set forth.

E. S. EARLEY.

Witnesses:

JOHN A. WIEDERSHEIM,  
A. P. GRANT.